

## 1

3,661,782

**HYDRAULIC BRAKE FLUID BASE OILS**  
 Malcolm K. Smith, Westfield, N.J., assignor to The Baker  
 Castor Oil Company, Bayonne, N.J.  
 No Drawing. Application Feb. 27, 1962, Ser. No. 176,126,  
 which is a continuation-in-part of application Ser. No.  
 690,417, Oct. 16, 1957, which in turn is a continuation-  
 in-part of application Ser. No. 629,585, Dec. 3, 1956.  
 Divided and this application Aug. 24, 1970, Ser. No.  
 66,554

Int. Cl. C09k 3/00

U.S. Cl. 252—79

5 Claims

**ABSTRACT OF THE DISCLOSURE**

Novel hydraulic brake fluids wherein the base oils are an adduct of a mixture of ethylene oxide and 1,2-propylene oxide with castor oil, and are characterized by having greatly improved properties, in connection with their use in brake fluids, over the properties of castor oil alone or in combination with either ethylene oxide or 1,2-propylene oxide.

This invention relates to base oils for hydraulic brake fluids and to brake fluids produced therefrom. The base oils of this invention are an adduct of a mixture of ethylene oxide and 1,2-propylene oxide with castor oil, and are characterized by having greatly improved properties, in connection with their use in brake fluids, over the properties of castor oil alone or in combination with either ethylene oxide or 1,2-propylene oxide.

This application is a division of application Ser. No. 176,126, filed Feb. 27, 1962, and now abandoned, which is a continuation-in-part of application Ser. No. 690,417, filed Oct. 16, 1957, now abandoned, which is a continuation-in-part of application Ser. No. 629,585, filed Dec. 3, 1956, now abandoned.

Hydraulic brake fluids are often subjected to extreme temperature variations and must be so constituted that they retain a relatively invariable viscosity, a homogeneous mixture and resist decomposition, solidification and separation of the ingredients throughout the temperature range to which they are exposed. Castor oil has proven to be deficient in several respects as a base oil for hydraulic brake fluids. These deficiencies include relatively poor low temperature properties, inadequate water tolerance, and relatively low viscosity indexes. Presently available synthetic base oils of the polyalkylene glycol type provide brake fluids characterized by having insufficient lubricity.

An object of this invention is to overcome these and other undesirable characteristics by providing base oils for hydraulic brake fluids which are characterized by improved low temperature properties, improved viscosity indexes, improved water tolerances, and improved lubricity, as well as surpassing the other established requirements for such base oils. Another object is to provide improved hydraulic brake fluids for heavy duty application containing the base oils of this invention. Other objects of this invention will be evident from the following specification.

In accordance with this invention it has been found that when mixtures of ethylene oxide and 1,2-propylene oxide are added to castor oil in predetermined proportions in a predetermined manner new and useful com-

## 2

positions are obtained which are characterized by stability at low temperatures. The products of this invention differ radically in their compositions from glycol and polyglycol esters of castor oil which have previously been suggested for use in hydraulic brake fluids. The products of this invention are for hydraulic use far superior to those glycol esters of castor oil, and as described below, exhibit excellent response to standard commercial tests: particularly as to complete or substantially complete lack of haze or opalescence after prolonged exposure to low temperatures.

The products of the invention are formed by sequentially reacting ethylene oxide with the castor oil and then reacting said mixture with the propylene oxide, or by 15 simultaneously reacting ethylene oxide and 1,2-propylene oxide with the castor oil, either by simultaneously adding the oxides separately to the castor oil or mixing the oxides prior to reaction with the castor oil.

Satisfactory products for use as base oils in this invention are those which are miscible with a minimum of 10% of water at room temperature, and which, in the form of a 20% solution by weight in 2-butoxyethanol, are characterized by having the ability to flow within 5 seconds and by being free from appreciable hazing after being maintained at —40° F. for 6 days.

In general, the satisfactory best products of this invention include the finished adduct containing from about 25% to about 45% by weight of a total mixed oxide component comprising about 90% ethylene oxide and about 10% propylene oxide; the finished adduct containing from about 25% to about 55% by weight of a total mixed oxide component comprising about 80% ethylene oxide and about 20% propylene oxide; the finished adduct containing from about 45% to 65% by weight of a total mixed oxide content comprising about 60% ethylene oxide to 40% propylene oxide. Satisfactory results are obtained when the reaction is carried out so that the products have compositions within the following limits:

|                 | Percent by weight |
|-----------------|-------------------|
| Castor oil      | 35-70             |
| Propylene oxide | 2½-50             |
| Ethylene oxide  | 5-50              |

For example, a product of particularly fine performance has a composition of 45% mixed oxides (60% ethylene, 40% propylene) and 55% castor oil.

Suitable diluents for use in the hydraulic brake fluids of this invention are organic oxygen-containing compounds selected from the group consisting of aliphatic monohydric, dihydric, and trihydric alcohols having from 1 to 7 carbon atoms and aliphatic ether alcohols having from 3 to 10 carbon atoms. Examples of diluents within this category include methyl alcohol, ethyl alcohol, propyl alcohols, butyl alcohols, amyl alcohols, diacetone alcohol, ethylene glycol, propylene glycol, methyl pentanediol, and dipropylene glycol, hexylene glycol, glycerine, 2-methoxyethanol, 2-ethoxyethanol, 2-butoxyethanol, methoxy-methoxyethanol, and the mono-methyl, mono-ethyl, and mono-butyl ethers of diethylene glycol.

The base oils of this invention have been found to have good compatibility, even at low temperatures, with diluents of the type listed above. Excellent brake fluids can be prepared by the use of 20% by weight of a base oil of this invention and 80% by weight of one or more of the foregoing diluents. Of course, the relative amounts of base

oil and diluent can be varied as desired, with a preferred amount of diluent being from about 60 to about 90 weight percent, based on the combined weight of the base oil and diluent.

The instant base oils have much lower viscosities at reduced temperatures than do the prior art unmodified esters. This fact results in an extension in the number of permissible diluents, including those with higher viscosities, over those which could previously be used. Some viscosity data on the base oils of this invention, as well as

- (7) Slight precipitate on bottom
- (8) Heavy precipitate on bottom
- (9) Phase separation
- (10) Solid or gelled

5 A passing rating in this test is from 1 to 3, with 3+ being on the borderline. It will be noted that hydraulic fluids containing the base oils of this invention (Examples 1-4, 6-12) pass this test without difficulty. The fluids containing base oils having too high a percentage of an oxide (Examples 5, 13), on the other hand, are not able to pass

TABLE II.—GOLD TEST DATA

| Example number                                                                                | 1   | 2   | 3   | 4   | 5  | 6   | 7   | 8  | 9                                                                                             | 10 | 11 | 12 | 13 |
|-----------------------------------------------------------------------------------------------|-----|-----|-----|-----|----|-----|-----|----|-----------------------------------------------------------------------------------------------|----|----|----|----|
| Base oils:                                                                                    |     |     |     |     |    |     |     |    |                                                                                               |    |    |    |    |
| Castor oil:                                                                                   |     |     |     |     |    |     |     |    |                                                                                               |    |    |    |    |
| 30% mixed adduct A <sup>1</sup>                                                               | 20  | 20  |     |     |    |     |     |    |                                                                                               |    |    |    |    |
| 40% mixed adduct A                                                                            |     | 20  | 20  |     |    |     |     |    |                                                                                               |    |    |    |    |
| 50% mixed adduct A                                                                            |     |     | 20  |     |    |     |     |    |                                                                                               |    |    |    |    |
| 30% mixed adduct B <sup>2</sup>                                                               |     |     |     | 20  | 20 |     |     |    |                                                                                               |    |    |    |    |
| 40% mixed adduct B                                                                            |     |     |     |     | 20 | 20  |     |    |                                                                                               |    |    |    |    |
| 50% mixed adduct B                                                                            |     |     |     |     |    | 20  | 20  | 20 |                                                                                               |    |    |    |    |
| 60% mixed adduct B                                                                            |     |     |     |     |    |     | 20  | 20 | 20                                                                                            |    |    |    |    |
| Diluents:                                                                                     |     |     |     |     |    |     |     |    |                                                                                               |    |    |    |    |
| Propylene glycol                                                                              |     |     |     |     |    |     |     |    | 20                                                                                            | 20 |    |    |    |
| 2-butoxyethanol                                                                               |     | 80  | 80  | 80  |    |     |     | 80 |                                                                                               | 80 | 80 |    |    |
| Celanese 901 H                                                                                |     |     |     |     |    |     |     |    |                                                                                               |    |    |    |    |
| n-Butanol                                                                                     | 80  | 80  |     |     |    |     | 80  |    | 80                                                                                            | 60 | 60 |    |    |
| 3-methyl butanol                                                                              |     |     |     |     |    |     |     |    |                                                                                               |    |    |    |    |
| Hexylene glycol                                                                               |     |     |     |     |    |     |     |    |                                                                                               |    |    |    |    |
| Methyl isobutyl carbinol                                                                      |     |     |     |     |    |     |     |    |                                                                                               |    |    |    |    |
| Cold test ratings                                                                             | 2-3 | 1-2 | 2-3 | 1-2 | 5  | 2-3 | 1-2 | 2  | 2-3                                                                                           | 2  | 2  | 2  | 5  |
| <sup>1</sup> 90% C <sub>2</sub> H <sub>4</sub> O, 10% C <sub>3</sub> H <sub>6</sub> O adduct. |     |     |     |     |    |     |     |    | <sup>2</sup> 80% C <sub>2</sub> H <sub>4</sub> O, 20% C <sub>3</sub> H <sub>6</sub> O adduct. |    |    |    |    |

on previously available ricinoleic acid esters, are presented in Table I.

TABLE I.—VISCOSITY DATA

| Base oil                                      | Kinematic viscosity, 0° F. (centistokes) | Viscosity index (A.S.T.M. D-567-53) | Pour point, ° F. |
|-----------------------------------------------|------------------------------------------|-------------------------------------|------------------|
| Castor oil                                    | Ca. 75,000                               | 84                                  | -10              |
| Blown castor oil (visc.: 23 stokes at 25° C.) |                                          | 95                                  | 0                |
| Ethylene glycol monoricinoleate               | Ca. 100,000                              | 65                                  | -5               |
| Propylene glycol monoricinoleate              | Ca. 100,000                              | 36                                  | -15              |
| Castor oil, 30% mixed adduct A <sup>1</sup>   | Ca. 12,000                               | 127                                 | -35              |
| Castor oil, 40% mixed adduct A <sup>1</sup>   |                                          |                                     | -35              |
| Castor oil, 50% mixed adduct A <sup>1</sup>   |                                          |                                     | -5               |
| Castor oil, 30% mixed adduct B <sup>2</sup>   |                                          |                                     | -35              |
| Castor oil, 40% mixed adduct B <sup>2</sup>   |                                          |                                     | -40              |
| Castor oil, 50% mixed adduct B <sup>2</sup>   | Ca. 10,000                               | 127                                 | -45              |
| Castor oil, 60% mixed adduct B <sup>2</sup>   |                                          |                                     | -15              |

<sup>1</sup> 90% C<sub>2</sub>H<sub>4</sub>O, 10% C<sub>3</sub>H<sub>6</sub>O adduct. <sup>2</sup> 80% C<sub>2</sub>H<sub>4</sub>O, 20% C<sub>3</sub>H<sub>6</sub>O adduct.

In general, the higher the viscosity index, the lower is the change of viscosity with temperature. Thus, high viscosity indexes parallel low viscosities at reduced temperatures. It will be noted that the instant base oils have desirably higher viscosity indexes than do the previously available esters. A rough correlation also exists between pour points of base oils and the abilities of hydraulic brake fluids containing the oils to pass the necessary cold tests. In general, the dividing line between acceptable and non-acceptable base oils appears to be in the vicinity of a pour point of -20° F. Most of the instant base oils have pour points at or below this dividing line, while the previously available esters do not. Some of the oxide adducts containing higher percentages of alkylene oxide have high pour points, and, as revealed by Table II, brake fluids containing these adducts fail to pass the cold test.

In Table II, data are presented on the results of cold tests run on hydraulic brake fluids containing base oils of this invention, as well as other base oils. This cold test is that prescribed by the Society of Automotive Engineers under the designation, S.A.E. 70R1. The hydraulic fluid under test is maintained at -40° F. for six days. At the end of that time, it should flow in five seconds and show no more than slight opalescence or hazing, and no stratification, or precipitation. The test ratings are based on visual observations, as follows:

- (1) Brilliant
- (2) Clear
- (3) Very slight haze, or slight opalescence
- (3+) Heavy opalescence
- (4) Slight precipitate through-out
- (5) Moderate precipitate through-out
- (6) Heavy precipitate through-out

30 Brake fluids should not attack and corrode the metals in the brake system. Hydraulic fluids containing the base oils of this invention have acceptable corrosion characteristics. Some typical data on this property are presented in Table III.

TABLE III

Corrosion data were obtained on the composition of Example No. 11 by the S.A.E. 70R1 procedure (immersion of metal strips in fluid for 5 days at 210° F.) with addition of—

|                             | .5 borax and .5 borax and .01 NaNO <sub>2</sub> | .5 borax and .01 KNO <sub>3</sub> |
|-----------------------------|-------------------------------------------------|-----------------------------------|
| Tinned iron (0.2 max. loss) | 0.1                                             | 0.003                             |
| Steel (0.2 max. loss)       |                                                 | 0.01                              |
| Aluminum (0.1 max. loss)    | 0.01                                            | 0.01                              |
| Cast iron (0.2 max. loss)   | 0.03                                            | 0.05                              |
| Brass (0.5 max. loss)       | 0.06                                            | 0.02                              |
| Copper (0.5 max. loss)      | 0.03                                            | 0.04                              |

45 Since small amounts of water may gain access to hydraulic fluid systems through condensation, leakage, or accident, it is essential that hydraulic fluids be miscible with minor percentages of water. In other words, the presence of water in the hydraulic system should not adversely affect the action of the brakes. The chemical incorporation of mixed oxides into castor oil results in greatly improved water miscibility over that of the unmodified oil. It has been found that, if the water miscibility of a base oil at room temperature is such that clear solutions result upon the incorporation of some 10 weight percent of water into the base oil, the base oils are eminently satisfactory with respect to this property. Base oils of this invention which have a suitable degree of water tolerance include, for example, adducts of castor oil containing a minimum of 30% of mixed oxides. The prior art unmodified oil and esters do not have water miscibilities approaching those of the base oils of this invention, and are quite unsatisfactory in this regard.

55 60 65 70 75 From the safety standpoint, it is important that hydraulic fluid base oils have high flash points. The flash points of the base oils of this invention are suitably high.

Because of the presence of rubber parts in brake systems, it is important that the base oils not cause rubber swelling beyond the acceptable maximum limits established by the Society of Automotive Engineers. When natural rubber cups are immersed in the fluid under test for five days at 158° F., the size of the cup should not change by more than 0.05 inch. The base oils of this invention have proved to be highly satisfactory in this respect.

In Table IV, the properties of a heavy duty brake fluid containing a base oil of this invention is compared with the heavy duty specification requirements established by the Society of Automotive Engineers. It will be observed that this hydraulic fluid meets the established requirements without difficulty, and especially that the viscosity at  $-40^{\circ}$  F. is far below the established maximum viscosity. This means that this hydraulic fluid can be utilized without difficulty at quite low operating temperatures.

TABLE IV.—PERFORMANCE OF HEAVY DUTY BRAKE FLUIDS

| S.A.E. 70R1 heavy duty specification requirements, base oil                        |                                                                                                                    |
|------------------------------------------------------------------------------------|--------------------------------------------------------------------------------------------------------------------|
| Boiling point ( $^{\circ}$ F.)                                                     | {300 $^{\circ}$ F. (minimum).<br>boiling point after 6 hrs.<br>(at 295 $^{\circ}$ F., 295 $^{\circ}$ F. (minimum). |
| Flash point                                                                        | Flash 145 $^{\circ}$ F. (minimum).                                                                                 |
| Viscosity (centistokes)                                                            | { $40^{\circ}$ F., 1,800 (max.).<br>(130 $^{\circ}$ F., 4.0 (min.).                                                |
| Cold test (5 second flow)                                                          | $-40^{\circ}$ F., at 6 days (no ppt. or strat.).                                                                   |
| Water tolerance (1 day) ( $140^{\circ}$ F. and $-40^{\circ}$ F.)                   | 5 sec. flow (no ppt. or strat.).                                                                                   |
| Neutrality (before and after corrosion test)                                       | {Before, pH 7 to 11.<br>After, pH 6 to 10.                                                                         |
| Compatibility ( $140^{\circ}$ F. and $-40^{\circ}$ F.)                             | No ppt. or strat.                                                                                                  |
| Evaporation percent                                                                | 210 $^{\circ}$ F. at 48 hours, 80% (max.).                                                                         |
| Residue test                                                                       | Liquid at 32 $^{\circ}$ F.<br>(158 $^{\circ}$ F. at 120 hours.                                                     |
| Rubber swell                                                                       | .005 (min.).<br>.050 (max.).                                                                                       |
| Corrosion loss (mg./cm. <sup>2</sup> ), 120 hours at $210^{\circ} + 5^{\circ}$ F.: |                                                                                                                    |
| Tinned iron                                                                        | .2 (Max.).                                                                                                         |
| Steel SAE 100                                                                      | .2 (Max.).                                                                                                         |
| Alum. SAE 24                                                                       | .1 (Max.).                                                                                                         |
| Cast iron SAE 111                                                                  | .20 (Max.).                                                                                                        |
| Brass SAE 70R                                                                      | .5 (Max.).                                                                                                         |
| Copper SAE 71                                                                      | .5 (Max.).                                                                                                         |

| Formulation of Example 14 <sup>1</sup>                                      | Example 14 <sup>1</sup> |
|-----------------------------------------------------------------------------|-------------------------|
| Boiling point:                                                              |                         |
| $^{\circ}$ F.                                                               | 325                     |
| After 6 hrs. at 295 $^{\circ}$ F. (295 $^{\circ}$ F. Min.)                  | 295                     |
| Flash point, degrees                                                        | 167                     |
| Viscosity (centistokes):                                                    |                         |
| $-40^{\circ}$ F., 1,800 max.                                                | 690                     |
| 130 $^{\circ}$ F., 4.0 min.                                                 | 5.5                     |
| Cold test (5 second flow) $40^{\circ}$ F., at 6 days.                       | 1-2                     |
| Water tolerance (1 day) ( $140^{\circ}$ F. and $-40^{\circ}$ F.) 5 sec flow | Pass                    |
| Neutrality (before and after corrosion test):                               |                         |
| Before pH 7 to 11.                                                          | 9.5                     |
| After, pH 6 to 10.                                                          | 7.7                     |
| Compatibility ( $140^{\circ}$ F. and $-40^{\circ}$ F.)                      | Pass                    |
| Evaporation (percent) at 210 $^{\circ}$ F. at 48 hrs.                       | 80                      |
| Residue test                                                                | Pass                    |
| Rubber swell (158 $^{\circ}$ F. at 120 hrs.)                                | .036                    |
| Corrosion loss (mg./cm. <sup>2</sup> ), 120 hrs. at $210 \pm 5^{\circ}$ F.: |                         |
| Tinned Iron                                                                 | .02                     |
| Steel SAE 100                                                               | .01                     |
| Alum. SAE 24                                                                | .02                     |
| Cast Iron SAE 111                                                           | .01                     |
| Brass SAE 70B                                                               | .00                     |
| Copper SAE 71                                                               | .00                     |

<sup>1</sup> See following table:

|                                                                  | Parts by weight |
|------------------------------------------------------------------|-----------------|
| Base oil, castor oil                                             | .20             |
| Propylene glycol, 40%                                            | .20             |
| Adduct of 2-butoxyethanol, 80% (C <sub>2</sub> H <sub>5</sub> O) | .60             |
| And borax, 20% (C <sub>3</sub> H <sub>6</sub> O)                 | .5              |

By way of summary, the base oils of this invention completely satisfy the many essential requirements of a satisfactory hydraulic fluid base. As indicated, the instant base oils are characterized by having low viscosities at reduced temperatures, high viscosity indexes, good water tolerance, and excellent lubricity. In addition, these oils are physically stable and chemically inert to an unusual degree, are miscible with a wide range of oxygen-containing organic diluents, have a negligible effect on rubber, have very low pour points, and are stable at elevated temperatures. As regards the high degree of lubricity of the instant base oils, this is an essential property of oils to be used in hydraulic brake fluids. Moving metal parts invariably form a part of the fluid transmission system, and a low frictional coefficient is necessary for ease of operation and for minimum abrasion and surface wear. In the lubrication tests

prescribed by the Society of Automotive Engineers, the base oils of this invention have been found to be without a peer of all those tested.

What is claimed is:

- An hydraulic brake fluid consisting essentially of: (a) a base oil which is an adduct of castor oil with a mixture of about 60% ethylene oxide and about 40% propylene oxide with the total mixed oxides being in the range of 25% to 65% by weight of the adduct, said adduct being characterized by having the ability to flow within 5 seconds and being substantially free from haze after being maintained at  $-40^{\circ}$  F. for six days; and (b) an organic oxygen containing alcohol diluent selected from the group consisting of aliphatic monohydric, dihydric, and trihydric alcohols having from 1 to 7 carbon atoms and aliphatic ether alcohols having from 3 to 10 carbon atoms.
- The fluid of claim 1, in which said diluent is present in an amount of from about 60 to about 90 weight percent, based on the combined weight of said adduct and diluent.
- An hydraulic brake fluid consisting essentially of; (a) a base oil which is an adduct of castor oil with a mixture of about 5% to about 50% by weight ethylene oxide, based on the total weight of the adduct, and about 2½% to about 50% by weight propylene oxide, based on the total weight of the adduct, said castor oil constituting about 40% to about 60% by weight of the adduct, and (b) a diluent selected from the group consisting of mono-(lower) alkylene glycols, di-(lower) alkylene glycols, lower alkyl ethers of said glycols, primary mono-hydric (lower) alcohols and secondary mono-hydric-(lower) alcohols.
- The fluid of claim 3, in which said diluent is present in an amount of from about 60 to about 90 weight percent, based on the combined weight of said adduct and diluent.
- An hydraulic brake fluid consisting essentially of: (a) a base oil which is an adduct of castor oil with a mixture of about 60% ethylene oxide and about 40% propylene oxide with the total mixed oxides being in the range of 25% to 45% by weight of the adduct, said adduct being characterized by having the ability to flow within 5 seconds and being substantially free from haze after being maintained at  $-40^{\circ}$  F. for six days; and (b) an organic oxygen containing alcohol diluent selected from the group consisting of aliphatic monohydric, dihydric, and trihydric alcohols having from 1 to 7 carbon atoms and aliphatic ether alcohols having from 3 to 10 carbon atoms.

#### References Cited

#### UNITED STATES PATENTS

|           |         |                    |             |
|-----------|---------|--------------------|-------------|
| 2,200,494 | 5/1940  | Fife               | 252—79      |
| 2,233,382 | 2/1941  | De Groot et al.    | 260—410.6 X |
| 2,451,999 | 10/1948 | Walker             | 252—79      |
| 2,469,285 | 5/1959  | White              | 252—78      |
| 2,588,970 | 3/1952  | Esposito           | 252—79      |
| 2,674,619 | 4/1954  | Lundsted           | 260—485     |
| 2,755,251 | 7/1956  | Barker             | 252—79      |
| 2,758,976 | 8/1956  | Barker             | 252—79      |
| 2,944,976 | 7/1960  | Waters et al.      | 252—79 X    |
| 2,987,490 | 6/1961  | Kirkpatrick et al. | 260—410.6 X |

#### FOREIGN PATENTS

|         |         |               |        |
|---------|---------|---------------|--------|
| 764,922 | 1/1959  | Great Britain | 252—79 |
| 876,007 | 8/1961  | Great Britain | 252—79 |
| 853,487 | 10/1952 | Germany       | 252—79 |

LEON D. ROSDOL, Primary Examiner

H. A. PITLICK, Assistant Examiner